# EUROPEAN PATENT APPLICATION

(11) **EP 4 700 165 A1**
(43) Date of publication of application: **25.02.2026**
(21) Application number: 24461612.4
(22) Date of filing: 21.08.2024
(51) Int. Cl.: D03D 9/00, D03D 13/00, D03D 27/06, D03D 27/10, E01C 13/08

(54) **A MAT FOR A HYBRID TURF**

(71) Applicant: Dywilan Sp. z o.o, 90-212 Lodz (PL)
(72) Inventor: JAKUBIAK, Piotr, 91-473 Lodz (PL); EJTASZEWSKI, Jacek, 90-701 Lodz (PL)
(74) Representative: Kancelaria Eupatent.pl Sp. z o.o.

(57) **Abstract**

A mat for a hybrid turf, having a base woven fabric, comprising pile burls interlaced with weft, wherein the ends of the burls form synthetic grass blades, the mat having a warp density from 54 to 72 ends/10cm, a weft density from 30 to 80 ends/10cm, and a pile height from 20 to 140 mm, wherein the total area of openings in the base fabric is from 5% to 15% of the total area of the base fabric of the mat, characterized in that the warp yarns (2) are made of biodegradable natural fibers having a linear mass from 100tex to 400tex, the weft yarns (5) are made of biodegradable natural fibers having a linear mass from 140tex to 1000tex, and the pile yarns (3, 4) are made of biodegradable natural fibers or biodegradable polymer yarns having a linear mass from 65tex to 1200tex.

## Description

### TECHNICAL FIELD

The invention pertains to a fully biodegradable mat for a hybrid turf and the hybrid turf made of it, which includes artificial grass and promotes the growth of natural grass.

### BACKGROUND

Turfs are generally categorized into natural turfs and artificial turfs. Natural turfs, where grass grows directly on soil, offer high comfort but are susceptible to damage under heavy use, requiring significant time to recover. Artificial turfs, composed entirely of synthetic materials, typically consist of an artificial mat with long blades of artificial grass protruding from it, with spaces between the blades filled with artificial granules. While artificial turfs are durable, they provide lower comfort compared to natural turfs.

Carpet based hybrid turfs, which combine a base mat with artificial grass covered by soil in which natural grass grows, are also known. The roots of the natural grass grow through the artificial base and integrate with it permanently. Over time, the natural grass blades grow above the level of the artificial grass blades, offering a comfort of use similar to that of natural turf. In high-use areas, such as the goal area on a soccer field, when the natural grass blades are damaged, the artificial grass blades become exposed, reducing comfort of use but not as significantly as in the case of damaged natural turfs.

Mats for hybrid turfs must provide appropriate base parameters, including permeability for water and air, and must also allow natural grass roots to grow through the base. The simplest known method to ensure appropriate base permeability is to perforate the base after installation, which complicates the installation process.

A European patent EP2698460B1 discloses a mat for a hybrid sport or decorative turf, having a form of a woven fabric, with a single-sided cover pile made of olefin synthetic yarns such as polyethylene and/or polypropylene and/or polyester, according to a 3/8W or 5/12W or 7/16W weave structure, comprising pile burls interlaced with weft, wherein the ends of the burls form synthetic grass blades. The mat has from 5000 to 20000 pile burls per square meter, a warp density from 54 to 72 ends/10cm, a weft density from 30 to 80 ends/10cm and a pile height from 20 to 140 mm, wherein each pile burl is interlaced at least two times over three weft yarns, and wherein the total surface mass of the mat is from 753 to 2105 g/m².

Existing hybrid turf mats face challenges related to installation complexity, base permeability, and integration with natural grass. These issues necessitate the development of alternative constructions for hybrid turf mats to address these challenges effectively.

### SUMMARY OF THE INVENTION

The aim of the invention is to provide a fully biodegradable, woven mat for a hybrid turf with a construction alternative to the known mats for hybrid turfs.

The use of biodegradable materials for the warp, weft, and pile yarns ensures that the mat will break down naturally over time, reducing environmental impact. This is particularly beneficial in applications where the mat may need to be replaced frequently, such as in high-use sports fields or decorative turfs in public spaces. The biodegradable nature of the mat means that it will not contribute to long-term waste, making it an environmentally friendly alternative to traditional synthetic mats.

The mat according to the invention is useful for hybrid sport or decorative turfs and is formed by a woven fabric comprising an artificial grass cover and a base through which roots of natural grass can easily grow. The mat has advantages of both artificial and natural turf, is resistant to adverse climatic conditions, and can withstand heavy use. If the mat is damaged, only the damaged fragments need to be replaced. The mat can be used to form turf systems in the final destination or on a plant site. The mat is highly flexible, even with the filling layer with natural grass, therefore it can be rolled up and transported in ready-to-install hybrid turf strips.

The mat comprises a base woven fabric, comprising pile tufts interlaced with weft, wherein the ends of the tufts form synthetic grass blades. The mat has a warp density from 54 to 72 ends/10cm, a weft density from 30 to 80 ends/10cm, and a pile height from 20 to 140 mm. The total area of openings in the base fabric is from 5% to 15% of the total area of the base fabric of the mat. The warp yarns are made of biodegradable natural fibers having a linear mass from 100tex to 400tex, the weft yarns are made of biodegradable natural fibers having a linear mass from 140tex to 1000tex, and the pile yarns are made of biodegradable natural fibers or biodegradable polymer yarns having a linear mass from 65tex to 1200tex.

The warp and weft yarns can be selected to have a shorter biodegradability period than the pile yarns. Preferably, the warp and weft shall disintegrate within 1-2 vegetation seasons. This ensures that the structural integrity of the mat is maintained during the initial growth period of the natural grass. As the warp and weft disintegrate, the remaining pile yarns still provide some structural support to the turf. This gradual disintegration process creates more openings for unrestricted growth of natural grass, enhancing the integration of the natural and artificial components of the hybrid turf. This feature is particularly advantageous compared to fully synthetic mats, which can impede the growth of natural grass due to their lack of biodegradability.

The warp yarns can be made of cotton (with a biodegradation time from 3 months to 2 years) and/or viscose (with a biodegradation time from 6 weeks to 2 years). The weft yarns can be made of jute (with a biodegradation time from 6 months to 2 years) and/or cotton (with a biodegradation time from 3 months to 2 years) and/or linen (with a biodegradation time from 6 months to 2 years) and/or hemp (with a biodegradation time from 6 months to 2 years). The pile yarns can be made of naturally colored cotton fibers (with a biodegradation time from 3 months to 2 years) or biodegradable polymer yarns (with a biodegradation time from 2 years to 6 years).

In case there is a need to increase the stability of the mat and resistance of tufts to pulling out, the bottom of the mat can be coated with a fixing water-based dispersion, for example in the amount of 50 to 120 g/m2 dry mass. The fixing dispersion shall be also biodegradable. The fixing dispersion used in the mat can be an aqueous solution of a natural binder, such as starch, with additional supplements that improve the growth of natural grass. This natural binder not only ensures the biodegradability of the mat but also contributes to the health and growth of the natural grass. The supplements can include nutrients and growth enhancers that provide the necessary elements for the grass to thrive. This dual functionality of the fixing dispersion - acting as both a binder and a growth supplement - further enhances the environmental benefits and practical utility of the mat.

The biodegradability of the mat also opens up a range of use applications. For instance, in temporary installations such as event venues or seasonal sports fields, the mat can be installed and then left to decompose naturally after the event or season is over. This eliminates the need for costly and labor-intensive removal and disposal processes. Additionally, the mat can be used in environmentally sensitive areas where the use of non-biodegradable materials would be inappropriate or prohibited.

The woven mat can have a single-sided cover pile made according to a 3/8W or 5/12W or 7/16W weave structure. Each pile tuft can be interlaced at least two times over three weft yarns. The mat may have from 5000 to 20000 pile tufts per m2, and the total surface mass of the mat can be from 753 to 2105 g/m2.

The mat, due to its loose structure, provides good conditions for the development of the root system of natural grass and permeability for water and air. The preferable warp density provides a loose structure of the mat with a pile linear mass of above 5000 dtex and, at the same time, it allows for openings in the base fabrics of the mat. Moreover, despite its loose character, the mat maintains a coherent structure even during use.

The fixation of the tufts, measured as the force necessary to pull out or break a blade, depending on the weave structure used and its density, may range from 17 to 74N. The fixation shall be large enough so that the mat does not need to be additionally coated by fixing dispersion at the bottom side and maintain maximal elasticity and permeability for water and air.

The coherency of the mat, which is particularly important for heavy use, for example when the mat is used on sports fields, can be achieved by the use of an interlaced arrangement of the binding yarn and the filling yarn between the pile yarn. At least one working yarn which forms the pile can be located between interlaced sets of three and six warp threads. Such an interlaced configuration of sets of three and six threads provides optimal stability of the weft yarns of the mat, while also providing adequate permeability for water and air in the mat, which can be at least 100,000 mmH2O/hour.

The openings in the base may be distributed uniformly and have a uniform size, for example of at least 25 mm², such that per each square centimeter of the base of the mat, in its initial state, i.e., before it is installed in the field, there can be openings having an area from 0.5 to 4 mm2. The openings in the mat may enlarge when grass roots grow through them, so that the threads surrounding the opening move aside under the force of the grass root, which is possible due to the loose structure of the mat.

In order to further stabilize the mat for the hybrid turf, the mat may comprise incorporated pile yarns, located preferably between the working pile yarn and the filling warp, which improve the dimensional stability of the mat. The linear mass of the working pile yarn forming the cover of the mat is from 80% to 120% of the linear mass of the incorporated pile yarn.

It is preferable to use pile threads having a total linear mass above 5000 dtex, more preferably above 6000 dtex and most preferably above 10000 dtex.

Multicolor yarns can be used as the pile, for example, multiple shades of green, which allows obtaining artificial grass tufts having a shade similar to that of natural grass. Therefore, the pile yarns can be made of at least two filaments. For example, the incorporated pile yarn may be formed by three filaments, each having a linear mass of 2000 dtex, and the working pile yarn may be formed by three filaments, each having a linear mass of 2000 dtex, which results in the total pile linear mass of 6000 dtex.

Use of the incorporated yarn in the base allows obtaining a mat having stable dimensions, with adequate parameters such as water and air permeability, and high uniformity of distribution of openings per each square centimeter, which allows use of the mat for creating hybrid sport or decorative turfs.

Finally, the mat is used to form a hybrid turf by laying the mat on a ground surface (such as of soil or sand subbase) and covering its top surface with a filling layer with grass seeds. As the grass seeds incubate, the roots of grass grow through the openings in the base layer towards the ground and the blades of natural grass grow atop the mat between the artificial blades. The filling layer can be any known permeable cultivating material, such as natural or synthetic sand, pozzolana, incinerator ash, organic particles, synthetic particles such as rubber particles, or mixtures thereof.

### BRIEF DESCRIPTION OF THE DRAWINGS

The object of the invention is shown in a drawing, in which:
Fig. 1 shows a mat according to the first embodiment, made according to a 3/8W weave structure,
Fig. 2 shows a mat according to the second embodiment, made according to a 7/16W weave structure,
Fig. 3 shows a bottom view of a mat according to the third embodiment, made with a 7/16W weave structure.

### DETAILED DESCRIPTION OF EMBODIMENTS

### First embodiment - Fig. 1.

The mat is constructed as a woven fabric using a 3/8W weave structure, particularly suitable for non-professional recreational areas, especially in regions with water scarcity. The mat comprises: working pile yarns and incorporated pile yarns made of 400 tex naturally colored cotton fibers; weft yarns made of 280 tex jute; and binding warp and filling warp yarns made of 200 tex cotton. The mat has a weft density of 36 ends/10cm and the length of yarn in a single burl is 86mm for a pile height of 35 mm.

The mat is made by interlacing the filling warp 1 and the binding warp 2 with the working pile yarn 3, the incorporated pile yarn 4, and the weft 5. The filling warp 1, the binding warp 2, the weft 5, and the incorporated pile yarn 4 form the base fabric. The working pile yarn 3 forms burls of artificial grass, wherein each burl is interlaced three times (as shown in Fig. 1) or seven times (as shown in Fig. 2) with the weft yarns 5 and two ends of the working pile yarn 3. The mat is made by double face weaving, wherein in a single process two mats are made: a top and a bottom mat, which are then separated by a cutting device integrated into the weaving machine. In the double face weaving, both fabrics are made of weft yarns 5, binding warp yarns 2, filling warp yarns 1, incorporated pile yarn 4, and working pile yarn 3, wherein the working pile yarns 3 are interlaced interchangeably in the top and the bottom fabric by weft yarns 5 according to a W weave structure, wherein each burl of artificial grass comprises two working pile yarn ends 3.

### Second embodiment - Fig. 2

The mat is constructed as a woven fabric using a 7/16W weave structure, suitable for professional soccer fields and other heavy-use applications. The mat comprises: working pile yarns and incorporated pile yarns made of 1000 tex biodegradable polymer; weft yarns made of 800 tex cotton; binding warp yarns and filling warp yarns made of 300 tex viscose. The mat has a weft density of 36 ends/10cm and the length of yarn in a single burl is 120mm for a pile height of 50 mm.

### Third embodiment - Fig. 3

Fig. 3 shows the distribution of individual threads as viewed from the bottom of the mat, which is made with a 7/16W weave structure. The mat has a yarn configuration comprising a binding warp 2, a filling warp 1, a working pile yarn 3, and an incorporated pile yarn 4, which are interlaced with a weft yarn 5. Each yarn of the incorporated pile yarn 4 is located between the working pile yarn 3 and the filling warp 1, wherein the incorporated pile yarn 4 is interlaced with the weft yarns 5 in the same manner as the yarns of the filling warp 1. The working pile yarn 3 is interlaced with the weft yarns 5 in the same manner as the binding warp yarns 2. The filling warp yarns 1 and the binding warp yarns 2 form a configuration of interchangeably positioned sets of three and six warp threads, between which, in the warp direction, there are positioned working pile yarns 3 and incorporated pile yarns 4. The set of six warp threads, looking from the left of the figure, comprises consecutively: two filling warp threads 1a, 1b, a binding warp 2c, a filling warp 1d, a binding warp 1e, and a filling warp 1f. The set of six warp yarns provides stability to the mat and maintains the position of the weft yarns 5 across the entire fabric area. The set of three warp threads comprises a filling warp 1g, a binding warp 2h, and a filling warp 1i. The set of warp threads allows the mat to have a total mat base layer mass of above 256 g/m² while maintaining high permeability for water, air, and grass root systems.

### Other embodiments

The mat may further comprise a configuration of two yarns: the working pile yarn 3 and the incorporated pile yarn 4, wherein the incorporated pile yarn 4 is optional. The pile yarns may extend in the warp direction, between the sets of three and six warp threads. The working pile yarn 3 may be interlaced with weft yarns 5 by a 7/16W weave structure. The ends of the working pile yarn 3 that extend outside the fabric form artificial grass burls, wherein each burl can be formed by two parallel yarns of the working pile yarns 3, extending in one row of pile yarns in the warp direction, the ends of which are output from the fabric at the same weft 5 (not shown in the drawing). The burls formed in this way create equal rows in the warp direction, but the burls of a pile in one row are shifted with respect to pile burls of parallel neighboring rows (i.e., the successive burls of artificial grass do not form parallel rows in the weft direction), which allows for a more even distribution of burls on the mat surface.

The incorporated pile yarn may extend between the threads of the working pile yarns 3 and between the sets of six or three warp threads such that each yarn of the incorporated pile yarn 4, which extends in parallel along one yarn of the working pile yarn 3 and the set of six weft yarns, in the place 6 of protrusion of two working pile yarns 3, changes its position and extends in parallel between the successive working pile yarn 3 and the set of three warp threads. Such a configuration of piles in the fabric provides stability to the dimensions of the mat.

## Claims

1. A mat for a hybrid turf, having a base woven fabric, comprising pile burls interlaced with weft, wherein the ends of the burls form synthetic grass blades, the mat having a warp density from 54 to 72 ends/10cm, a weft density from 30 to 80 ends/10cm, and a pile height from 20 to 140 mm, wherein the total area of openings in the base fabric is from 5% to 15% of the total area of the base fabric of the mat, **characterized in that** the warp yarns (2) are made of biodegradable natural fibers having a linear mass from 100tex to 400tex, the weft yarns (5) are made of biodegradable natural fibers having a linear mass from 140tex to 1000tex, and the pile yarns (3, 4) are made of biodegradable natural fibers or biodegradable polymer yarns having a linear mass from 65tex to 1200tex.

2. The mat according to claim 1, wherein the warp yarns (2) are made of cotton and/or viscose.

3. The mat according to any of the previous claims, wherein the weft yarns (5) are made of one or more of: jute, cotton, linen and hemp yarns.

4. The mat according to any of the previous claims, wherein the pile yarns (3, 4) are made of naturally colored cotton and/or biodegradable polymer.

5. The mat according to claim 1, **characterized in that** its bottom is coated with biodegradable fixing water-based dispersion with natural grass nutrients and/or growth enhancers.

6. The mat according to claim 1, **characterized in that** the weft yarns (5), the warp yarns (2), and the pile yarns (3, 4) are movable to form openings of a size of at least 25 mm².

7. The mat according to claim 1, **characterized in that** it comprises at least one opening having an area from 0.5 mm² to 4 mm² per each square centimeter of the area of the base fabric of the mat.

8. The mat according to claim 1, **characterized in that** it further comprises incorporated pile yarn (4).

9. The mat according to claim 4, **characterized in that** each yarn of the incorporated pile yarn (4) is located between the working pile yarn (3) and the filling warp (1).

10. The mat according to claim 1, **characterized in that** the total linear mass of the working pile yarns (3) from 80% to 120% of the linear mass of the incorporated pile yarn.

11. The mat according to claim 1, **characterized in that** the working pile yarn (3) is made of at least two filaments.

12. The mat according to claim 1, **characterized in that** at least one working pile yarn (3) is located between interlaced sets of three and six warp threads (1, 2).

13. The mat according to claim 12, **characterized in that** between the interlaced sets of three and six warp threads (1, 2) there is further located an incorporated pile yarn (4).

14. The mat according to claim 12, **characterized in that** the set of three warp threads comprises consecutively a filling warp (1g), a binding warp (2h), and a filling warp (1i) and the set of six warp threads comprises consecutively two filling warp threads (1a, 1b), a binding warp (2c), a filling warp (1d), a binding warp (1e), and a filling warp (1f).

15. The mat according to claim 12, **characterized in that** the burls of a pile (3) in each row are shifted with respect to pile burls (3) of parallel neighboring rows.
